

Sept. 19, 1967

TADASHI NEMOTO ET AL

3,342,058

ROLL FOR COLD-ROLLING METALLIC SHEET MATERIALS

Original Filed March 25, 1963

2 Sheets-Sheet 1

Fig. 1



Fig. 3



INVENTORS

Tadashi Nemoto  
Toshiya Yaegashi

By Paul M. Ensign, Jr.  
ATTORNEY

Sept. 19, 1967

TADASHI NEMOTO ET AL

3,342,058

ROLL FOR COLD-ROLLING METALLIC SHEET MATERIALS

Original Filed March 25, 1963

2 Sheets-Sheet 2

Fig. 2a  
Non-etching



Fig. 2b  
Etching with 10% nitric acid

MICROSTRUCTURE OF THE INVENTIVE ALLOY (x360)  
(Oil-quenched at 950°C)

INVENTORS

TADASHI NEMOTO  
TOSHIO YAGASHI

BY

*Paul M. Craig, Jr.*

ATTORNEY

1

3,342,058  
ROLL FOR COLD-ROLLING METALLIC  
SHEET MATERIALS

Tadashi Nemoto, Takahagi-shi, and Toshio Yaegashi, Hitachi-shi, Japan, assignors to Hitachi, Ltd., Tokyo, Japan, a corporation of Japan  
Continuation of application Ser. No. 267,757, Mar. 25, 1963. This application Oct. 28, 1966, Ser. No. 590,437

Claims priority, application Japan, Mar. 26, 1962,  
37/11,036  
2 Claims. (Cl. 72—365)

This application is a continuation of application Ser. No. 267,757 filed Mar. 25, 1963, now abandoned.

The present invention relates to roll materials and more particularly to those for use in the making of hardened forging-steel rolls and has for its object to provide a roll material of the type which is highly improved in hardenability and wear resistance.

Customarily, rolls of the Sendzimir mill for cold rolling have been made of a high-carbon high-chromium steel, which has heretofore been recommended, since the material when quenched from higher temperatures forms a martensite including chromium carbide of high hardness and thus has a substantial wear resistance. Most recently, however, the demand for improvements in dimensional accuracy and surface luster of rolled steel sheets has been increasing. Conventional roll materials such as high-carbon high-chromium alloy steels have been unable to meet this demand due to the lack of any satisfactory wear resistance.

In view of the above difficulty, the present invention is designed to furnish a roll material having an extraordinarily high wear resistance and a high hardenability.

According to the present invention, there is provided a roll material comprising from 1.0% to 2.5% by weight of carbon, 3% to 10% by weight of chromium, 0.5% to 8% by weight of molybdenum, 0.5% to 6% by weight of tungsten, 1.0% to 7.0% by weight of vanadium, not more than 0.5% by weight of silicon, and not more than 0.5% by weight of manganese, the balance being substantially iron.

Composition limits for each of the alloying elements will now be detailed.

Carbon forms carbides in the alloy, which are critically important for obtaining a desired wear resistance. However, less than 1.0% by weight of carbon gives only insufficient hardness and wear resistance while over 2.5% by weight of carbon impairs the hardenability of the alloy and reduces its ductility.

Chromium combines with carbon to form the carbides  $M_3C$  and  $M_7C_3$ , which are very hard, and thus plays an important role in enhancing the wear resistance of the roll. However, as the weight percentage of chromium decreases below 3%, the amount of these carbides is rapidly reduced. In the range of over 10% by weight, an excess of primary crystals of chromium carbide appears in masses to cause exfoliation or firecracking during use of the roll. Therefore, the chromium percentage must be coordinated with the proportions of the other alloying elements.

Molybdenum also forms carbides, while a part thereof forms a solid solution in the base contributing to the strength and the heat resistance at elevated temperatures. This is important since, particularly in Sendzimir mills, the surface temperature of the rolls is momentarily raised to a substantial extent requiring a substantially high strength in the base of the roll material. This effect of the presence of molybdenum rapidly decreases as the weight percentage is reduced below 0.5%. On the other hand, as the percentage increases, the amounts of molybdenum and

2

its carbide increase to give a highly improved wear resistance; however, in the range of over 8% both the workability and the hardenability of the alloy steel are markedly reduced.

Tungsten has substantially the same effects as molybdenum except that it raises the wear resistance of the alloy to a much greater extent than molybdenum. However, as the tungsten content exceeds 6% by weight, the amount of tungsten forming a solid solution in the base is increased, thereby making the roll fragile.

The use of vanadium is particularly significant in the present invention. In most of the high-carbon high-chromium steels previously used, chromium carbide in primary crystals is nonuniformly distributed in masses along the grain boundaries and such masses do not disappear even by subsequent working or heat treatment of the material, causing exfoliation or firecracking in the use of the roll formed of such material. Experiments have shown, however, that vanadium, if added together with chromium, forms a carbide during solidification in advance of chromium and in the form of minute spheroids to limit precipitation of the chromium carbide and thus prevents any nonuniform distribution of carbides in the alloy, as will clearly be observed in FIG. 2 in the accompanying drawing.

FIG. 2 represents two micrographs x360 of one example of the alloy according to the invention, which comprises 2.2% by weight of C, 0.3% by weight of Si, 0.6% by weight of Mn, 5.1% by weight of Cr, 0.85% by weight of Mo, 0.9% by weight of W, and 4.8% by weight of V, the rest being substantially iron. FIG. 2a, is a micrograph of a nonetched specimen oil-quenched at 950° C., showing clearly defined grains of vanadium carbide, while FIG. 2b, represents a micrograph of a specimen oil-quenched at the same temperature and etched with a 10% solution of nitric acid, showing that the formation of chromium carbide is effectively suppressed. Vanadium carbide is much harder than chromium carbide (about three times as hard as the latter) and thus is generally very effective in increasing the wear resistance of the roll. However, it is noted that the effect of the addition of vanadium is reduced to about one half as its weight percentage is reduced below 1% while the presence of vanadium in percentages of over 7% reduces the workability and hardenability of the alloy to a substantial extent.

The advantages of the roll material of the invention over the high-carbon high-chromium steel conventionally used as a roll material will be evident from FIG. 1, which graphically illustrates the relationship between the hardness and the quenching temperature of the two materials, and Table 1, which includes data comparing the two materials with respect to their wear resistance as expressed in terms of their resistance to grinding. The composition of the roll material according to this invention forth hereinbefore in connection with FIG. 2. On the other hand, the high-carbon high-chromium steel selected as a typical example of conventional roll material comprised 2.1% by weight of C, 12.5% by weight of Cr, 0.85% by weight of Mo, and 0.88% by weight of V, the balance being substantially iron. In FIG. 1, the solid line represents the hardness of the alloy of the invention while the dotted line represents that of the conventional high-carbon high-chromium steel. As observed in this figure, the alloy of the invention has an optimum quenching temperature lower than that of the high-carbon high-chromium steel, thereby facilitating the hardening procedure to that extent. It has been found in this testing that the alloy of the invention has a satisfactory self-hardenability and exhibits excellent mechanical properties due to its fine-grained structure as seen in the micrographs of FIG. 2.

The data in Table 1 were obtained employing a grinding wheel of Japanese Industrial Standard WA-46-1 on a plane grinder. Specimens of the inventive and conventional alloy steels were prepared in a size of 10 mm. (c) x 10 mm. (d) x 80 mm. (e) (see FIG. 3) and ground at a peripheral speed of 1600 mm./min. for comparing the two materials with respect to their wear resistance.

TABLE 1

| Material of specimen    | Weight, gr.             |                          | Weight ratio,<br>$\frac{B}{A} \times 100\%$ | Specific<br>wear<br>resistance |
|-------------------------|-------------------------|--------------------------|---------------------------------------------|--------------------------------|
|                         | Material removed<br>(A) | Grit<br>dislodged<br>(B) |                                             |                                |
| High-C high-Cr steel... | 8.220                   | 0.321                    | 2.56                                        | 1                              |
| Inventive alloy-----    | 7.357                   | 0.528                    | 7.18                                        | 2.8                            |

As apparent from this table, the alloy of the invention exhibits a notably reduced grindability compared with the conventional roll material and is duly expected to have a wear resistance nearly three times as high as that of the latter. Actual use of rolls formed of the alloy of the invention in a rolling mill for non-ferrous alloys and in a small-sized Sendzimir mill has demonstrated the fact that the alloy gives a highly improved roll performance compared with any of the conventional roll materials.

We claim:

1. In a process of cold-rolling metals by means of a rolling mill having rolls which contact the metal, the improvement in said process comprising contacting said metals with said rolls, said rolls consisting essentially of

25

1.0 to 2.5% by weight of carbon, 3 to 10% by weight of chromium, 0.5 to 8% by weight of molybdenum, 0.5 to 6% by weight of tungsten, 1.0 to 7% by weight of vanadium, not more than 0.5% by weight of silicon, not more than 0.6% by weight of manganese, the balance being substantially iron and a small amount of impurities.

2. In a process of cold-rolling metals by means of a rolling mill having rolls which contact the metal, the improvement in said process comprising contacting said metals with said rolls, said rolls consisting essentially of 10 2.2% by weight of carbon, 0.3% by weight of silicon, 0.6% by weight of manganese, 5.1% by weight of chromium, 0.85% by weight of molybdenum, 0.9% by weight of tungsten, 4.8% by weight of vanadium, and the balance being substantially iron.

15

## References Cited

## UNITED STATES PATENTS

|    |           |        |                  |        |
|----|-----------|--------|------------------|--------|
| 20 | 2,174,286 | 9/1939 | Gill -----       | 75—126 |
|    | 2,736,650 | 2/1956 | Grimshaw -----   | 75—126 |
|    | 2,867,532 | 1/1959 | Payseen -----    | 75—126 |
|    | 2,983,601 | 5/1961 | Fletcher -----   | 75—126 |
|    | 2,996,376 | 8/1961 | Nehrenberg ----- | 75—126 |

## OTHER REFERENCES

Roberts et al.: Tool Steels, 3rd ed., Apr. 16, 1962, pub. by the American Society for Metals, pp. 237 and 238,

30 HYLAND BIZOT, Primary Examiner.

P. WEINSTEIN, Assistant Examiner.